

Patented Nov. 2, 1926.

1,605,192

## UNITED STATES PATENT OFFICE.

PAUL McALLISTER, OF BLOOMFIELD, NEW JERSEY, ASSIGNOR TO WESTINGHOUSE LAMP COMPANY, A CORPORATION OF PENNSYLVANIA.

## PROCESS FOR PRODUCING NONSAG TUNGSTEN WIRE.

No Drawing.

Application filed December 23, 1922. Serial No. 608,796.

This invention relates to incandescent electric lamps and, more particularly, to a process for producing a non-sag tungsten filament for use in such lamps.

5 An object of the invention is to provide a process for rendering a normally non-sag wire more resistant to sagging.

A further object of the invention is to maintain a normally non-sag lamp filament 10 in a condition to resist sagging throughout its normally useful life.

Another object of the invention is the provision of a step in the fabrication of a non-sag tungsten lamp filament whereby 15 harmful compounds or substances within the filament may be rendered harmless to prevent any deleterious action on the non-sag properties thereof.

A still further object of the invention is 20 to subject a wire to the action of a strong reducing agent, such as arsenic or phosphorus, and, conjunctively therewith, intensively heating said wire, whereby deleterious substances within said wire may be 25 rendered harmless.

Other objects of the invention will be apparent upon a reading of the following description.

Processes have been devised for obviating 30 the tendency of coiled filaments of incandescent electric lamps of the gas-filled type to elongate or sag between supports, when burned at high temperatures, by producing a pure tungsten filament. According to 35 these processes, it is proposed to add to the tungsten powder a purifying substance, as the nitrates or carbonates of potassium or sodium, silicic acid, etc. It was thought that these processes would have the effect 40 of purifying the tungsten and removing therefrom any deleterious substances which may subsequently affect the crystal development in said wire.

However, in the wire which is produced 45 in accordance with these processes, it is found that there still may be included within the wire objectionable compounds either resulting from the materials which have been added to the wire or which said materials have failed to remove during the process of fabrication of the material into a wire or filament.

I have determined by examination of numerous filaments that it is a condition prec-

edent to obtaining a good non-sag wire 55 that the wire be physically homogeneous. The filament should be in this condition at the time the lamp is first burned or else if not present at that time it is necessary that such condition be developed at that time 60 and that it be thus maintained throughout the life of the lamp.

I have also discovered that grain size or shape do not determine of themselves the sag-resisting qualities of a wire. Also I 65 have discovered that it is not necessary in the production of a non-sag wire that any particular auxiliary ingredients or doping materials be added to the wire. As stated heretofore, my tests and examinations of 70 various so-called non-sag wire have revealed that that quality which a wire must possess in order to render the same resistant to sagging is physical homogeneity at the time or immediately after the wire is first lighted 75 as a filament. In order that this property may be possessed by the wire at the time mentioned, it is necessary that there be removed from the wire those substances which affect the crystalline structure adversely, 80 and if the wire is introduced into a lamp as a filament, it is also a condition that any materials present in the lamp, which may form harmful compounds with the filament, be rendered harmless.

With the end in view, therefore, of providing a filament which is physically homogeneous at the beginning of the life of the wire as a filament, I have ascertained that this condition may be developed by subjecting the wire, after its manufacture, to the action of a strong reducing agent, such as arsenic, phosphorus and the like. It is a condition that the reducing agent be of such nature that it will remove moisture, oxygen or harmful substances or compounds from the surface of the filament or within the filament itself or the surrounding atmosphere in which said filament may be burned. The reducing agent also should have a low 100 boiling point so that it does not remain in the wire as an impurity.

Several methods may be followed in subjecting the wire to the action of the reducing agent. A desirable method may consist in inserting the wire into, or passing it slowly through, an enclosed vessel or tube furnace provided with an inert environment, such as

argon, nitrogen and the like. The reducing agent may be introduced into the furnace in the form of a vapor, either with or independently of the inert gas. It may be desirable, however, to apply the reducing agent to the wire in the form of a coating by passing the wire through a liquid such as water containing the reducing agent in suspension. In the latter case, the reducing agent may be rendered active by heating the wire to incandescence by passing an electrical current therethrough or the wire may be heated in any other desired manner. It is preferable to heat the wire to a high temperature while the reducing agent is active as the beneficial action in removing impurities or rendering them harmless is expedited thereby.

It may be desirable, however, from the practical and commercial aspect to subject the wire to the reducing action after it has been inserted into the lamp. However, in the latter case the material which is to act as the reducing agent must be in such condition that its action will not be impaired. It also may be desirable that the reducing agent be active throughout the normal commercially useful life of the lamp, therefore, a sufficient quantity of the agent may be placed within the lamp to enable this continuous action to be maintained, it being a condition, however, that the reducing agent employed be such that it has an appreciable vapor pressure at the lowest temperature prevailing within the lamp during operation thereof.

In order that the beneficial action of the reducing agent upon the filament may be rendered more effective, it may be found desirable to conjunctively heat the filament to a high temperature at the time the reducing agent is rendered active. To this end it may be preferable to apply the reducing agent directly to the lamp filament.

By comparison of the two sets of data hereinafter given, the reader may better appreciate the benefits derived by employment of my invention. Four lamps containing coils of tungsten wire made in accordance with the standard process for producing non-sag wire, were seasoned for 15 minutes at 100% voltage and for 45 minutes at 115% voltage. These lamps, after seasoning, were tested in various ways. They showed an average bump test of 23, an average strength of coil of 10.2 and an average sag of 1.7 mm.

Another set of lamps were made up containing wire from the same spool. These lamps, however, were subjected to the action of a strong reducing agent and thereafter were tested in the same fashion as the previous lamps. The bump test for these lamps showed an average of 63, an average strength of coil of 21.1 and an average sag of 1 mm.

It is obvious from a comparison of these averages that the lamps which were subjected to the action of a strong reducing agent showed a marked improvement over the lamps made from the same lot of wire and which were not subjected to such an agent. An examination of the micro photographs of the wire which was subjected to the strong reducing agent discloses a structure which was physically homogeneous. The wire from the other lamps, however, showed numerous crystal groups which interrupted and destroyed the physical continuity of the metal.

Although I have specified certain materials as being desirable reducing agents, it is obvious that there are many other substances which may act in this capacity, for example, sulphur, lithium, sodium, potassium, rubidium and caesium, as well as other low-boiling-point substances, may be employed. The best results have been obtained, however, by employing arsenic or phosphorus.

I am aware of a patent which describes the application of phosphorus to the lamp filament and the activation thereof after the lamp has been tipped-off. However, in such patent, the process claimed therein and the description relate to lamps of a different type from those which I contemplate improving, that is, such process relates to vacuum lamps. It is well known that, in a vacuum lamp, a condition is met which deterioriously affects the filament after the lamp has been burned some time, namely the offsetting of the filament. In order to prevent offsetting, it is the practice to incorporate with the filament a material such as thoria or other high-melting-point substance.

I have found that, when the strong reducing agent is applied to a filament of this character, no material improvement is effected in the properties of the filament, so far as making the same resistant to sagging, as the quantity of the offset-resisting material employed is so large that the reducing agent is incapable of rendering the same harmless. In lamps of the type to which my invention is applicable, the filaments are formed of tungsten to which has been added no offset-resisting material. In other words, the filament is formed of substantially pure tungsten.

It is to be appreciated that departures from the invention may be obvious to those skilled in the art, however, I contemplate including such modifications as fall within the scope of the appended claims.

What is claimed is:

1. The step in the production of substantially non-sag tungsten which consists in flashing tungsten in the presence of a low-boiling point reducing agent to remove substances from the tungsten which affect the

continuity of the tungsten structure and thereby produce a continuous tungsten structure.

2. The step in the production of a substantially non-sag tungsten wire which consists in flashing in the presence of a reducing agent a tungsten wire containing substances affecting the continuity of the tungsten structure to remove such substance from the wire and thereby produce a continuous tungsten structure.

3. The method of treating a tungsten wire of the non-sag type to render the same more resistant to sagging and of greater strength, which comprises flashing in the presence of a reducing agent, a tungsten wire of the non-sag type to remove from said wire, substances affecting the continuity of the tungsten structure, and maintaining said continuous tungsten structure by surrounding the same with a reducing agent capable of combining with substances which would affect the continuity of the tungsten structure if combined therewith.

25 4. The step in the production of substantially non-sag tungsten which consists in flashing the tungsten in phosphorus to remove substances from the tungsten which affect the continuity of the tungsten structure and thereby produce a continuous tungsten structure.

30 5. The step in the production of a substantially non-sag wire which consists in flashing, in the presence of phosphorus and the like, a tungsten wire containing substances affecting the continuity of the tungsten structure to remove such substances from the wire and thereby produce a continuous tungsten structure.

35 40 6. The method of treating a tungsten wire of the normally non-sag type to render the same more resistant to sagging and of greater strength which comprises flashing, in the presence of phosphorus and the like, a tungsten wire of the non-sag type to remove from said wire, substances affecting the continuity of the tungsten structure, and main-

50 taining said continuous tungsten structure by surrounding the same with a reducing agent capable of combining with substances which would affect the continuity of the structure if combined therewith.

55 7. The method of improving the non-sag and strength qualities of a tungsten wire of the normal non-sag type which comprises hermetically sealing the same in an enclosing vessel and subjecting the wire to the action of a low boiling point reducing agent and simultaneously heating the wire, the reducing agent being in sufficient quantity to act upon substances capable of deleteriously affecting the wire throughout a commercially useful life of the device.

60 8. A tungsten filament substantially resistant to sagging and of improved strength consisting of a plurality of grains or crystals of tungsten in intimate contact and having no substances between or within the grain boundaries affecting the continuity of the tungsten structure.

65 70 9. A tungsten filament substantially resistant to sagging and of improved strength comprising a substantially clean tungsten intercrystalline structure.

10. An incandescent lamp having a filament therein substantially resistant to sagging and of improved strength, said filament consisting of substantially clean intercrystalline tungsten free from substances affecting the continuity of the tungsten structure.

75 80 11. An incandescent lamp having a filament therein substantially resistant to sagging throughout a commercially useful life, said filament consisting of substantially clean intercrystalline tungsten free from substances affecting the continuity of the tungsten structure, and a low boiling reducing agent within said lamp capable of protecting said filament to prevent its continuity being destroyed.

85 90 In testimony whereof, I have hereunto subscribed my name this 21st day of December 1922.

PAUL McALLISTER.